# EUROPEAN PATENT SPECIFICATION

(11) **EP 3 901 312 B1**
(45) Date of publication and mention of the grant of the patent: **18.10.2023**
(21) Application number: 19899913.8
(22) Date of filing: 01.11.2019
(51) Int. Cl.: C22C 38/34, C22C 38/22, C22C 38/28, C22C 38/26, C22C 38/32, C22C 38/04, C22C 38/06, C22C 38/24, C22C 38/00, C21D 8/02, C22C 38/02

(54) **HIGH STRENGTH HOT-ROLLED STEEL SHEET HAVING EXCELLENT WORKABILITY, AND METHOD FOR MANUFACTURING THE SAME**
HOCHFESTES WARMGEWALZTES STAHLBLECH MIT AUSGEZEICHNETER BEARBEITBARKEIT UND VERFAHREN ZUR HERSTELLUNG DAVON
FEUILLE D'ACIER LAMINÉE À CHAUD À HAUTE RÉSISTANCE PRÉSENTANT UNE EXCELLENTE APTITUDE AU FAÇONNAGE, ET SON PROCÉDÉ DE FABRICATION

(30) Priority: 18.12.2018 KR 20180163898
(43) Date of publication of application: 27.10.2021
(73) Proprietor: POSCO Co., Ltd, Pohang-si, Gyeongsangbuk-do 37859 (KR)
(72) Inventor: NA, Hyun-Taek, Gwangyang-si, Jeollanam-do 57807 (KR); KIM, Sung-Il, Gwangyang-si, Jeollanam-do 57807 (KR); BAE, Gyu-Yeol, Incheon 21985 (KR)
(74) Representative: Meissner Bolte Partnerschaft mbB
(86) International application number: PCT/KR2019/014669
(87) International publication number: WO 2020/130329

(56) References cited:
- EP-A1- 0 997 548
- EP-A1- 3 276 030
- EP-A1- 3 395 992
- WO-A1-2018/110853
- WO-A1-2018/179387
- CN-A- 108 950 423
- JP-A- 2005 298 956
- JP-A- 2005 298 956
- JP-A- 2010 138 421
- KR-A- 20010 020 169
- KR-A- 20180 068 099

## Description

### [Technical Field]

The present invention relates to a steel material which may be used for arms, frames, beams, brackets, reinforcements of chassis components of vehicles, and more particularly, to a high strength hot-rolled steel sheet having excellent workability, and a method for manufacturing the same.

### [Background Art]

A hot-rolled steel sheet is for example disclosed in WO 2018/179387 A1. Recently, demand for an increase in fuel efficiency of internal combustion engine vehicles and reductions in the weight of transportation engines, due to the weight of batteries in electrical vehicles, has been continuously increased. Also, automotive chassis components have been designed to have a reduced thickness according to higher strength. To secure safety of passengers by the reduction of thickness, steel sheets having been developed to date may exceed 750 MPa and 980 MPa grades in terms of tensile strength, and development of a high strength steel sheet of 1180 MPa grade has been necessary. However, in the case of simply increasing strength based on the techniques having developed so far, formability such as elongation and hole expandability may degrade, which may be problematic.

A technique for securing excellent elongation by the phenomenon of transformation induced plasticity (TRIP) by forming retained austenite in a structure to secure formability for a high strength steel sheet has been developed (References 1 to 3). The main features of these techniques are to secure elongation by forming relatively coarse and equiaxed crystal-shaped retained austenite on a certain fraction of polygonal ferrite and high-angle grain boundaries in a microstructure

However, when a component is processed, retained austenite may be easily transformed into martensite by the above-mentioned transformation induced plasticity phenomenon, such that, due to a large difference in hardness with polygonal ferrite, hole expandability, which represents burring properties close to an actual formability mode, may greatly degrade when chassis components are processed.

To overcome this, a technique of securing elongation and hole expandability by reducing a difference in phase hardness between retained austenite and a low-temperature ferrite, or between retained austenite and bainite by increasing fractions of the low-temperature ferrite and bainite in a steel sheet has been developed(Reference 4).

However, to prevent transformation of polygonal ferrite, the technique may include a method of rapid cooling after rolling, such that an additional cooling facility device may be inevitable, which may cause a limitation in productivity, and it may not be easily to uniformly secure various physical properties such as strength in a coil and hole expandability due to rapid cooling immediately after rolling.

### [Prior Art Document]

### [Reference]

(Reference 1) Japanese Laid-Open Patent Publication No. 1994-145894
(Reference 2) Japanese Laid-Open Patent Publication No. 2008-285748
(Reference 3) Korean Laid-Open Patent Publication No. 10-2012-0049993
(Reference 4) Japanese Laid-Open Patent Publication No. 2012-251201
(Reference 5) WO 2018/179387 A1

### [Disclosure]

### [Technical Problem]

An aspect of the present invention is to provide a hot-rolled steel sheet having high strength and excellent formability of elongation and hole expandability, and a method for manufacturing the same.

### [Technical Solution]

Solution to the above-described technical problem is provided in the independent claims.

### [Advantageous Effects]

A hot-rolled steel sheet in the present invention may have advantages of having excellent strength and also excellent formability. Therefore, using the hot-rolled steel sheet of the present invention, high strength and a reduced thickness may be obtained with respect to vehicle chassis components.

### [Brief Description of Drawings]

FIG. 1 is a graph illustrating a distribution of a product (TSXEl) of tensile strength and elongation, and a product (TSXHER) of tensile strength and hole expandability of inventive examples and comparative examples respectively in the present Example;
FIGS. 2(a) and (b) are images of microstructures of inventive example 7 and comparative example 2 respectively in the present Example; and
FIGS. 3 (a), (b), and (c) are diagrams illustrating a relationship between retained austenite and precipitates in a structure adjacent to the retained austenite of comparative example 14, inventive example 7 and comparative example 15 respectively in the present Example.

### [Best Mode for Invention]

General transformation induced plasticity (TRIP) steel may be applied to vehicle components requiring high ductility during forming components, and may be required to have a reduced thickness of less than 2.5 mmt level due to characteristics of the components. For this reason, cold rolling may be performed after hot rolling, and thereafter, a structure may be formed through a heat treatment process of an annealing process in which temperature and a speed of passing sheet may be controlled in a stable manner relatively. However, when the steel is used for chassis components as in the present disclosure, generally, a thickness may be in a range of 1.5-5 mmt, and in some cases, the thickness may be greater than this, such that it may not be suitable to manufacture the components by cold rolling. Also, the chassis components may need to secure ductility and also excellent hole expandability when a steel sheet is manufactured, and thus, retained austenite may need to be appropriately formed metallurgically, and it may be also necessary to reduce a difference in hardness between retained austenite and a matrix structure. The present disclosure has been devised to overcome the above-described technical difficulties, to implement TRIP properties for a hot-rolled steel sheet, and to secure excellent hole expandability.

In the description below, the present disclosure will be described in greater detail.

An alloy composition of the hot-rolled steel sheet of the present invention will be described in detail. The hot-rolled steel sheet of the present disclosure includes, by weight%, 0.1-0.15% of C, 2.0-3.0% of Si, 0.8-1.5% of Mn, 0.001-0.05% of P, 0.001-0.01% of S, 0.01-0.1% of Al, 0.7-1.7% of Cr, 0.0001-0.2% of Mo, 0.02-0.1% of Ti, 0.01-0.03% of Nb, 0.001-0.005% of B, 0.1-0.3% of V, 0.001-0.01% of N, and a balance of Fe and inevitable impurities.

### Carbon (C): 0.1-0.15 weight% (hereinafter, referred to as %)

C may be the most economical and effective for strengthening steel. When the amount of added C is increased, a fraction of bainite may increase, such that strength may increase, and the formation of retained austenite may be facilitated, which may be advantageous in securing an elongation based on a transformation induced plasticity effect. However, when the content is less than 0.1%, fractions of bainite and retained austenite may not be sufficiently secured during cooling after hot rolling, and formation of polygonal ferrite may occur by a decrease in hardenability. When the content exceeds 0.15%, strength may excessively increase due to an increase of a fraction of martensite, and weldability and formability may be deteriorated. Therefore, the content of C is 0.1-0.15%.

### Silicon (Si): 2.0-3.0%

Si may deoxidize molten steel and may contribute to an increase in strength through a solid solution strengthening effect. Also, Si may inhibit the formation of carbides in a structure and may facilitate the formation of retained austenite during cooling. However, when the content is less than 2.0%, the effect of inhibiting the formation of carbides in the structure and securing stability of retained austenite may be reduced. When the content exceeds 3.0%, ferrite transformation may be excessively promoted, such that fractions of bainite and retained austenite in the structure may rather decrease, and it may be difficult to secure sufficient physical properties. Also, red scale may be formed by Si on the surface of the steel sheet, such that the surface of the steel sheet may be deteriorated and weldability may be deteriorated, which may be problematic. Therefore, the content of Si is 2.0-3.0%.

### Manganese (Mn): 0.8-1.5%

Similarly to Si, Mn may be effective in solid solution strengthening of steel, and may improve hardenability of steel such that bainite or retained austenite may be easily formed during cooling after hot rolling. However, when the content is less than 0.8%, the above effect may not be obtained by the addition of Mn, and when the content exceeds 1.5%, a fraction of martensite may increase, and also the segregation region may be greatly developed in a center of a thickness during slab casting in a continuous casting process such that formability may degrade, which may be problematic. Therefore, the content of Mn is 0.8-1.5%.

### Phosphorus (P): 0.001-0.05%

P may be one of impurities present in steel, and when the content thereof exceeds 0.05%, ductility may decrease due to micro-segregation and impact properties of steel may degrade. To manufacture steel with less than 0.001% of P, it may take a lot of time and effort in steelmaking operation, which may greatly reduce productivity. Therefore, the P content is 0.001-0.05%.

### Sulfur (S): 0.001-0.01%

S may be one of impurities present in steel, and when the content thereof exceeds 0.01%, S may be combined with manganese and may form non-metallic inclusions, and accordingly, toughness of the steel may significantly degrade. To manage the content to be less than 0.001%, it may take a lot of time and effort in steelmaking operation, which may greatly reduce productivity. Therefore, the content of S is 0.001-0.01%.

### Aluminum (Al): 0.01-0.1%

Aluminum (preferably, Sol.Al) may be mainly added for deoxidation, and preferably, 0.01% or more of Al may be added to expect a sufficient deoxidation effect. However, when the content exceeds 0.1%, which is excessive, Al may be bonded with nitrogen such that AlN may be formed, and slab corner cracks may be likely to be formed during continuous casting, and defects may occur due to the formation of inclusions . Therefore, preferably, the content may be 0.1% or less. Thus, the content of Al is 0.01-0.1%.

### Chrome (Cr): 0.7-1.7%

Cr may solid-solution strengthen steel and, similarly to Mn, may delay phase transformation of ferrite during cooling such that Cr may contribute to forming bainite and retained austenite. To obtain the above effect, preferably, 0.7% or more of Cr may be added. However, when the content exceeds 1.7%, an elongation rate may decrease rapidly due to an excessive increase in phase fractions of bainite and martensite. Therefore, the Cr content is 0.7-1.7%.

### Molybdenum (Mo): 0.0001-0.2%

Mo may increase hardenability of steel such that formation of bainite may be facilitated. To this end, preferably, 0.0001% or more of Mo may be added. However, when the content exceeds 0.2%, hardenability may increase such that martensite may be formed, which may lead to degradation of formability and may be disadvantageous in terms of economic efficiency and weldability. Therefore, the content of Mo is 0.0001-0.2%.

### Titanium (Ti): 0.02-0.1%

Ti may be a representative precipitation enhancing element along with Nb and V, and may forms coarse TiN in steel with strong affinity with N. TiN may contribute to inhibiting growth of crystal grains during a heating process for hot rolling. Ti remaining after reacting with N may be dissolved in steel and may be bonded with carbon such that TiC precipitates may be formed, and TiC precipitates may improve strength of steel. To obtain the technical effect in the present disclosure, preferably, Ti may be added in an amount of 0.02% or more. However, when the content exceeds 0.1%, precipitation of TiN or TiC may be excessive, such that the solid solution C content required for formation of bainite and retained austenite in steel may decrease rapidly, and hole expandability may decrease. Therefore, the content of Ti is 0.02-0.1%.

### Niobium (Nb): 0.01-0.03%

Nb may be a representative precipitation strengthening element along with Ti and V. Nb may be precipitated during hot rolling and may refine crystal grains by delaying recrystallization, such that strength and impact toughness of steel may improve. To obtain the above effect, preferably, Nb may be added in an amount of 0.01% or more. However, when the content exceeds 0.03%, the solid solution C content in steel during hot rolling may be rapidly reduced, such that it may be impossible to secure sufficient bainite and retained austenite, and due to excessive delay of recrystallization, elongated crystal grains may be formed, which may deteriorate formability. Therefore, the content of Nb is 0.01-0.03%.

### Boron (B): 0.001-0.005%

B may be effective in securing hardenability of steel, and when B is present in a solid solution state, B may stabilize grain boundaries, such that brittleness of steel in a low-temperature region may improve. Also, B may form BN along with solid solution N, such that formation of coarse nitride may be prevented. To obtain the effect, preferably, 0.001% or more of B may be included. When the content exceeds 0.005%, recrystallization behavior may be delayed during hot rolling and a precipitation strengthening effect may be reduced. Therefore, the content of B is 0.001-0.005%.

### Vanadium (V): 0.1-0.3%

V may be a representative precipitation enhancing element along with Ti and Nb, and may improve strength of steel by forming precipitates after coiling. To obtain the effect, 0.1% or more of V may be added preferably. When the content exceeds 0.3%, coarse composite precipitates may be formed, such that formability may degrade, which may be economically disadvantageous. Therefore, the content of V is 0.1-0.3%.

### Nitrogen (N): 0.001-0.01%

N may be a representative solid solution strengthening element along with carbon, and may form coarse precipitates along with Ti and Al. Generally, a solid solution strengthening effect of nitrogen may be higher than that of carbon, but since toughness may decrease significantly when the amount of nitrogen in the steel increases, preferably, N may be added in an amount of 0.01% or less. To manufacture steel with the content of N to be less than 0.001%, it may take a lot of time for steelmaking operation, such that productivity may degrade. Therefore, the content of N is 0.001-0.01%.

A remainder includes Fe and inevitable impurities. In a range in which the technical effect of the present disclosure is not impaired, alloy components which may be additionally included in addition to the above-described alloy components may not be excluded.

Preferably, the alloy composition in the hot-rolled steel sheet of the present disclosure satisfies [relational expression 1] and [relational expression 2] as below. $\begin{matrix}20 \leq H γ \leq 50 \\ \begin{matrix}Hγ & =\end{matrix} \\ 194.5 - \left(\begin{matrix}428 \left[C\right] + 11 \left[Si\right] + 45 \left[Mn\right] + 35 \left[Cr\right] - 10 \left[Mo\right] - 107 \left[Ti\right] - 56 \left[Nb\right] - 70 \\ \left[V\right]\end{matrix}\right)\end{matrix}$

In relational expression 1, [elemental symbol] indicates a content (weight%) of each element.

In relational expression 1, Hγ is a relational expression of an effect of securing retained austenite stability by adding C, Si, Mn, Cr, Mo, Nb, and V, which are hardenability enhancing elements and an effect of reducing a difference in hardness between retained austenite and a matrix structure adjacent to retained austenite having precipitates in grains of the structure, by adding the elements.

In relational expression 1, when Hγ is less than 20, a hardenability effect may be high such that stability of retained austenite may be secured, but due to concentration of excessive alloy components in a retained austenite grain, retained austenite may be rapidly hardened. For this reason, a difference in hardness between retained austenite and ferrite, or between retained austenite and bainite may increase, and hole expandability of the steel sheet may be deteriorated. When Hγ exceeds 50, precipitates may be excessively formed in a structure adjacent to retained austenite, such that carbon content in the retained austenite may be insufficient, and stability of the retained austenite may be deteriorated, which may degrade elongation.

Preferably, to form an appropriate fraction of a precipitate in a structure adjacent to retained austenite, [relational expression 2] is satisfied in addition to [relational expression 1]. $\begin{matrix}0.7 \leq {a}_{p} \leq 3.5 \\ {a}_{p} = \left(\left[Mo\right]+\left[Ti\right]+\left[Nb\right]+\left[V\right]\right) \times {\left[C\right]}^{- 1}\end{matrix}$

In relational expression 2, [elemental symbol] indicates a content (weight%) of each element.

When a value of aₚ is less than 0.7, sufficient precipitates may not be formed in a structure adjacent to retained austenite, and when the value exceeds 3.5, precipitation may be excessive such that stability of the aforementioned retained austenite may be deteriorated.

A microstructure of the hot-rolled steel sheet of the present invention includes, by an area fraction, 5-15% of ferrite, 5-20% of retained austenite, and 10% or less of inevitable structure, in addition to bainite as a matrix structure. The inevitable structure may include martensite, a martensite austenite constituent (MA), or the like, and a sum of thereof does not exceed 10%. When the sum exceeds 10%, elongation may be deteriorated due to a decrease in a fraction of retained austenite, and also hole expandability may be deteriorated due to a difference in hardness between retained austenite and ferrite, or between retained austenite and bainite.

When a fraction of ferrite is less than 5%, most of elongation of the steel sheet may be dependent on retained austenite, such that it may be difficult to secure a level of elongation targeted in the present disclosure. When the content exceeds 15%, it may be difficult to secure sufficient strength. When the retained austenite is less than 5%, a fraction of an excessive low-temperature transformation phase such as martensite in a microstructure may increase, such that it may be easy to secure strength, but elongation may be deteriorated. When a fraction of retained austenite exceeds 20%, stability may be deteriorated due to a decrease in the carbon content in each retained austenite, and accordingly, most of the structure may be stress induced-transformed into martensite in an initial stage of deformation, such that ductility may degrade.

Preferably, an average hardness value of ferrite may be 200 Hv or more. When hardness value is less than 200 Hv, hole expandability may degrade due to a high difference in hardness between bainite and retained austenite. To secure the average hardness value of the ferrite, it may be important to secure a fraction of low angle grain boundary fraction, dislocation density, and precipitates in the ferrite, and to this end, a design of components of the steel sheet and also an optimized process may be necessary when the steel sheet is manufactured.

Preferably, in the hot-rolled steel sheet of the present disclosure, the number of precipitates having a diameter of 5 nm or more in ferrite present within 100µm from a retained austenite grain boundary in the microstructure may be 5×10ⁿ/mm² (1≤n≤3). When the number of precipitates is less than an effective range, the effect of reducing a difference in hardness between retained austenite and the structure adjacent to retained austenite may be insufficient, such that it may be difficult to secure hole expandability. When the number of precipitates exceeds an effective range, a fraction of retained austenite and bainite may degrade due to excessive precipitation, such that strength and ductility may be deteriorated.

The type of the precipitate is not particularly limited, and may be a carbide, nitride, or the like, including Mo, Ti, Nb, and V.

Preferably, the hot-rolled steel sheet of the present disclosure may have tensile strength (TS) of 1180 MPa or more, a product (TS×El) of tensile strength and elongation may be 20,000 MPa% or more, and a product (TS×HER) of tensile strength and hole expandability may be 30,000 MPa% or more.

In the description below, an example of manufacturing the present invention hot-rolled steel sheet will be described in detail. The hot-rolled steel sheet of the present disclosure is manufactured through a process comprising the steps of heating a steel slab satisfying the above-described alloy composition-hot rolling the heated steel slab-cooling the hot rolled steel sheet-coiling the cooled steel sheet. In the description below, each of the above processes will be described in detail.

A steel slab having the above-described alloy composition is prepared, and the steel slab is heated to a temperature of 1180-1300°C. When the heating temperature is less than 1180°C, heat of the steel slab may be insufficient such that it may be difficult to secure the temperature during hot rolling, and it may be difficult to remove segregation via diffusion generated during continuous casting. Also, precipitates precipitated during continuous casting may not be sufficiently re-solid solute, such that it may be difficult to obtain a precipitation strengthening effect in a process after hot rolling. When the content exceeds 1300°C, strength may be reduced and a structure may be formed non-uniformly due to coarse growth of austenite grains, and thus, the slab heating temperature is 1180-1300°C.

The heated steel slab is hot-rolled. Hot rolling the heated steel slab is started in a temperature range equal to or higher than a ferrite phase transformation initiation temperature (Ar3), and a hot finishing rolling temperature is managed within a temperature range satisfying [relational expression 3] as below: $\begin{matrix}900 \leq T * \leq 960 \\ T * = T + 225 {\left[C\right]}^{0.5} + 17 \left[Mn\right] - 34 \left[Si\right] - 20 \left[Mo\right] - 41 \left[V\right]\end{matrix}$ (where "T" indicates a hot finishing rolling temperature (FDT), and [elemental symbol] indicates a content (weight%) of each element).

When the finishing temperature after the rolling is less than the range of the relational expression 3, a fraction of coarse and elongated ferrite may increase, such that it may be difficult to secure target strength and formability. When the range of the relational expression 3 is exceeded, strength may degrade due to formation of a coarse structure at a high rolling temperature, and scaling surface defects may increase, such that formability may degrade from another viewpoint.

T* may be an effective temperature range for inhibiting formation of coarsely elongated ferrite by phase transformation in a two phase region which may occur before or during rolling. When an alloying element that delays ferrite transformation such as C or Mn is added, a range thereof may increase, but when the content of Si that promotes ferrite transformation increases, the range may decrease. Also, Mo and V may increase hardenability during phase transformation, similarly to C and Mn, but Mo and V may facilitate formation of carbides by bonding with C, and C which is necessary to form bainite and retained austenite may be exhausted through the formation of carbides, such that physical properties suggested in the present disclosure may not be secured. Accordingly, when T* is less than 900, a fraction of the elongated coarse ferrite may be high, such that a fraction of bainite and uniformity of distribution behavior of retained austenite may degrade, which may degrade strength and formability. When 960 is exceeded, a high-temperature heating operation may be inevitable to secure a high rolling temperature, such that scaling defects may occur, which may deteriorate surface quality, and a coarse structure may be formed, such that it may be difficult to secure strength and formability.

The hot-rolled steel sheet is cooled at a cooling rate of 20-400°C/s to a temperature range of 500-600°C (primary cooling) . When the primary cooling termination temperature is less than 500°C, which is rapid cooling, the steel sheet may be rapidly cooled in a transition boiling temperature range, which may shape and material uniformity may degrade. When 600°C may be exceeded, a fraction of polygonal ferrite may excessively increase, such that it may be difficult to secure sufficient strength and hole expandability. When the primary cooling rate exceeds 400°C/s, there may be a limitation in operation of a facility, and a shape and material uniformity may degrade due to non-uniformity of ferrite and bainite transformation behavior for the excessive cooling rate. When the cooling is performed at a cooling rate of less than 20°C/s, phase transformation of ferrite and pearlite may occur during the cooling, such that a desired level of strength and hole expandability may not be secured. The primary cooling rate may be more preferably 70-400°C/s.

After the primary cooling, if necessary, to increase low-temperature ferrite formation and a precipitation effect, a process of Extremely slow cooling at a cooling rate of 0.05-4.0°C/s for 12 seconds or less may be further included. When the Extremely slow cooling exceeds 12 seconds, it may be difficult to control the cooling in an actual run out table (ROT) section, and it may be difficult to secure desired fractions of bainite and retained austenite due to an increase in an excessive increase of fraction of ferrite in the structure, such that it may be difficult to secure desired properties.

After the primary cooling, cooling (secondary cooling) is performed at a cooling rate of 0.5-70°C/s to a temperature range of 350-500°C. In some cases, an Extremely slow cooling process may be included in the secondary cooling process. When the secondary cooling termination temperature is less than 350°C, fractions of martensite and MA phase may excessively increase, and when the temperature exceeds 500°C, fractions of bainite and retained austenite phase may not be secured, such that elongation and hole expandability may not be secured simultaneously at tensile strength of 1180 MPa or more. When the secondary cooling rate is less than 0.5°C/s, ferrite may be excessively formed, such that bainite and retained austenite may not be sufficiently secured, and it may be difficult to secure strength, and hole expansion may degrade due to a difference in hardness between phases. When the cooling rate exceeds 70°C/s, a fraction of bainite may increase and fractions of ferrite and retained austenite may decrease, such that it may be difficult to secure elongation. The secondary cooling rate may be more preferably 0.5-50°C/s.

The hot-rolled steel sheet on which the secondary cooling has been completed is coiled at the same temperature. Natural cooling may be performed on the coiled hot-rolled steel sheet to a temperature range of room temperature-200°C, and shape leveling may be carried out through leveler and surface layer scale may be removed by pickling or a process similar to pickling. When the temperature of the steel sheet exceeds 200°C, shape leveling may be easy during leveler, but roughness of the surface layer may be deteriorated due to over-pickling during pickling.

Also, a plated layer may be formed if necessary. The type and method of the plating are not particularly limited. However, to inhibit releasing of low-temperature transformation phases such as bainite and retained austenite during the heat treatment of the steel sheet, such as the heating for plating, the heat treatment may be performed at less than 600°C preferably.

### [Best Mode for Invention]

Hereinafter, the present invention will be described in greater detail through embodiments. However, it should be noted that the embodiment are merely to specify the present invention. The scope of the present invention is defined in the appended claims.

### (Example)

A steel slab having the alloy composition (weight%, a remainder is Fe and inevitable impurities) as in Table 1 was manufactured, was heated to 1250°C, was rough-rolled, was hot-rolled to 2.5-3.5mmt in a range in which a finishing temperature satisfies [relational expression 3], and was cooled under cooling conditions as in Table 2, thereby manufacturing a hot-rolled steel sheet. In this case, the cooling rate during the secondary cooling was controlled to be within 0.5-70°C/s, and the cooling was performed to the secondary cooling termination temperature as in Table 2, coiling was performed. Thereafter, natural cooling was performed in the air to room temperature, and shape leveling may be carried out through leveler and surface layer scale may be removed by pickling process.

For the hot-rolled steel sheet manufactured as above, a microstructure was observed using a scanning electron microscope (SEM), an area fraction was calculated using an image analyzer, and results thereof are listed in Table 3. In particular, an area fraction of an MA phase was measured using an optical microscope and an SEM at the same time after etching by the LePera etching method.

Particularly, the carbon content of retained austenite (RA) and a structure adjacent to retained austenite, and the distribution of the precipitates of the structure adjacent to retained austenite(RA) were specified using a transmission electron microscope (TEM), and in both the invention examples and comparative examples, the number of precipitates was an average value of precipitates having a diameter of 5 nm or more for 500 nm², 10 regions.

As for the rolling direction of the manufactured hot-rolled steel sheet, a JIS No. 5 standard sample was prepared with reference to 90° and 0° directions, a tensile test was performed at room temperature at a strain rate of 10mm/min, and yield strength (YS), tensile strength (TS) and elongation (El) were measured, which may indicate 0.2% off-set yield strength, tensile strength and fracture elongation, respectively. Yield strength and tensile strength were results of evaluating a 90° sample in the rolling direction, and elongation was a result of evaluating a 0° sample in the rolling direction. The tensile strength and elongation are listed in Table 3 below.

As for hole expandability (HER), a square sample of about 120mm in width and length was prepared, and a hole of a diameter of 10mm was punched in a center of the sample through punching operation, a burr was disposed upward, a cone was pushed up, and a diameter of the hole immediately before cracks were created in a circumferential region for a minimum hole diameter (10mm) was calculated in percentage and are listed in Table 3.

**[Table 1]**

| Class ifica tion | Composition (wt.%) | | | | | | | | | | | | | Rel ati ona l exp res sio n 1 | Rel ati ona l exp res sio n 2 |
|---|---|---|---|---|---|---|---|---|---|---|---|---|---|---|---|
| | C | Si | Mn | P | S | Al | Cr | Mo | Ti | Nb | B | V | N | | |
| Inven tive examp le 1 | 0.1 4 | 2.4 | 1.4 | 0.0 1 | 0.0 03 | 0.0 4 | 1.1 | 0.1 1 | 0.0 3 | 0.0 21 | 0.0 03 | 0.1 2 | 0.0 03 | 20. 6 | 2.0 |
| Inven tive examp le 2 | 0.1 2 | 2.4 | 1.1 | 0.0 1 | 0.0 03 | 0.0 4 | 1.4 | 0.0 5 | 0.0 3 | 0.0 15 | 0.0 04 | 0.1 2 | 0.0 04 | 31. 2 | 1.8 |
| Inven tive examp le 3 | 0.1 1 | 2.4 | 0.9 | 0.0 1 | 0.0 03 | 0.0 4 | 1.4 | 0.0 5 | 0.0 4 | 0.0 15 | 0.0 02 | 0.1 2 | 0.0 03 | 45. 5 | 2.0 |
| Inven tive examp le 4 | 0.1 3 | 2.1 | 1.3 | 0.0 1 | 0.0 03 | 0.0 4 | 1.1 | 0.1 5 | 0.0 3 | 0.0 15 | 0.0 03 | 0.1 1 | 0.0 04 | 32. 0 | 2.3 |
| Inven tive examp le 5 | 0.1 4 | 2.2 | 1.1 | 0.0 1 | 0.0 03 | 0.0 4 | 1.4 | 0.0 7 | 0.0 5 | 0.0 21 | 0.0 03 | 0.1 4 | 0.0 03 | 28. 9 | 2.0 |
| Inven tive examp le 6 | 0.1 4 | 2.4 | 1.4 | 0.0 1 | 0.0 03 | 0.0 4 | 0.8 | 0.1 4 | 0.0 3 | 0.0 21 | 0.0 02 | 0.1 2 | 0.0 03 | 31. 4 | 2.2 |
| Inven tive examp le 7 | 0.1 1 | 2.1 | 1.2 | 0.0 1 | 0.0 03 | 0.0 4 | 1.1 | 0.0 03 | 0.0 3 | 0.0 15 | 0.0 03 | 0.1 3 | 0.0 03 | 45. 0 | 1.6 |
| Inven tive examp le 8 | 0.1 4 | 2.9 | 0.9 | 0.0 1 | 0.0 03 | 0.0 4 | 1.4 | 0.0 03 | 0.0 4 | 0.0 15 | 0.0 03 | 0.1 9 | 0.0 03 | 31. 6 | 1.8 |
| Inven tive examp le 9 | 0.1 2 | 2.3 | 1.1 | 0.0 1 | 0.0 03 | 0.0 4 | 1.6 | 0.0 7 | 0.0 4 | 0.0 15 | 0.0 02 | 0.1 1 | 0.0 04 | 25. 9 | 2.0 |
| Compa rativ e examp le 1 | 0.2 4 | 2.1 | 0.9 | 0.0 1 | 0.0 03 | 0.0 4 | 1.1 | 0.1 5 | 0.0 3 | 0.0 15 | 0.0 03 | 0.0 9 | 0.0 04 | 1.5 | 1.2 |
| Compa rativ e examp le 2 | 0.0 8 | 2.2 | 1.1 | 0.0 1 | 0.0 03 | 0.0 4 | 1.1 | 0.1 5 | 0.0 3 | 0.0 15 | 0.0 01 | 0.1 1 | 0.0 03 | 61. 3 | 3.8 |
| Compa rativ e examp le 3 | 0.1 3 | 3.4 | 1.4 | 0.0 1 | 0.0 03 | 0.0 4 | 1.1 | 0.1 5 | 0.0 4 | 0.0 15 | 0.0 03 | 0.1 4 | 0.0 03 | 16. 4 | 2.7 |
| Compa rativ e examp le 4 | 0.1 3 | 1.8 | 0.9 | 0.0 1 | 0.0 03 | 0.0 4 | 1.1 | 0.0 5 | 0.0 4 | 0.0 15 | 0.0 02 | 0.1 2 | 0.0 04 | 54. 1 | 1.7 |
| Compa rativ e examp le 5 | 0.1 3 | 2.2 | 1.7 | 0.0 1 | 0.0 03 | 0.0 4 | 1.1 | 0.0 7 | 0.0 4 | 0.0 15 | 0.0 03 | 0.1 1 | 0.0 04 | 13. 2 | 1.8 |
| Compa rativ e examp le 6 | 0.1 3 | 2.9 | 0.6 | 0.0 1 | 0.0 03 | 0.0 4 | 1.1 | 0.0 7 | 0.0 4 | 0.0 15 | 0.0 03 | 0.0 9 | 0.0 03 | 53. 6 | 1.7 |
| Compa rativ e examp le 7 | 0.1 3 | 2.1 | 1.1 | 0.0 1 | 0.0 03 | 0.0 4 | 1.8 | 0.1 5 | 0.0 4 | 0.0 15 | 0.0 02 | 0.1 4 | 0.0 04 | 19. 7 | 2.7 |
| Compa rativ e examp le 8 | 0.1 3 | 2.4 | 1.1 | 0.0 1 | 0.0 03 | 0.0 4 | 0.5 | 0.1 5 | 0.0 3 | 0.0 15 | 0.0 02 | 0.0 9 | 0.0 04 | 57. 3 | 2.2 |
| Compa rativ e examp le 9 | 0.1 4 | 2.2 | 1.1 | 0.0 1 | 0.0 03 | 0.0 4 | 1.1 | 0 | 0.0 1 | 0.0 05 | 0.0 02 | 0.0 9 | 0.0 03 | 30. 0 | 0.8 |
| Compa rativ e examp le 10 | 0.1 4 | 2.1 | 1.1 | 0.0 1 | 0.0 03 | 0.0 4 | 1.1 | 0.2 2 | 0.1 1 | 0.0 35 | 0.0 03 | 0.3 1 | 0.0 03 | 61. 1 | 4.8 |
| Compa rativ e examp le 11 | 0.1 3 | 2.4 | 1.1 | 0.0 1 | 0.0 03 | 0.0 4 | 1.4 | 0.0 7 | 0.0 3 | 0.0 15 | 0.0 03 | 0.1 1 | 0.0 03 | 26. 4 | 1.7 |
| Compa rativ e examp le 12 | 0.1 4 | 2.1 | 1.1 | 0.0 1 | 0.0 03 | 0.0 4 | 1.1 | 0.0 7 | 0.0 3 | 0.0 15 | 0.0 03 | 0.1 2 | 0.0 03 | 36. 6 | 1.7 |
| Compa rativ e examp le 13 | 0.1 4 | 2.1 | 1.1 | 0.0 1 | 0.0 03 | 0.0 4 | 1.1 | 0.0 7 | 0.0 3 | 0.0 15 | 0.0 03 | 0.1 2 | 0.0 04 | 36. 6 | 1.7 |
| Compa rativ e examp le 14 | 0.1 4 | 2.1 | 1.1 | 0.0 1 | 0.0 03 | 0.0 4 | 1.1 | 0.0 7 | 0.0 3 | 0.0 15 | 0.0 03 | 0.1 2 | 0.0 04 | 36. 6 | 1.7 |
| Compa rativ e examp le 15 | 0.1 4 | 2.1 | 1.1 | 0.0 1 | 0.0 03 | 0.0 4 | 1.1 | 0.0 7 | 0.0 3 | 0.0 15 | 0.0 03 | 0.1 2 | 0.0 03 | 36. 6 | 1.7 |

(Relational expression 1 is Hγ = 194.5-(428[C]+11[Si]+45[Mn]+35[Cr]-10[Mo]-107[Ti]-56[Nb]-70 [V]), and relational expression 2 is aₚ - ([Mo]+[Ti]+[Nb]+[V])×[C]⁻¹)

**[Table 2]**

| Class ifica tion | FDT(T) (°C) | Relat ional expre ssion 3 | Primary cooling | | Extremely slow cooling | | Second ary coolin g | |
|---|---|---|---|---|---|---|---|---|
| | | | Termi natio n tempe ratur e | Cooli ng rate | Intermediat e temperature | Time | Termin ation temper ature | |
| | | T* | (°C) | (°C/s) | (°C) | (sec) | (°C) | |
| Inven tive examp le 1 | 931 | 950 | 591 | 85 | - | - | 453 | |
| Inven tive examp le 2 | 941 | 950 | 562 | 95 | - | - | 409 | |
| Inven tive examp le 3 | 948 | 950 | 561 | 97 | 555 | 6 | 481 | |
| Inven tive examp le 4 | 922 | 946 | 563 | 90 | 559 | 8 | 452 | |
| Inven tive examp le 5 | 929 | 950 | 582 | 87 | 577 | 8 | 466 | |
| Inven tive examp le 6 | 935 | 954 | 568 | 92 | 562 | 8 | 479 | |
| Inven tive examp le 7 | 931 | 949 | 564 | 92 | 557 | 6 | 443 | |
| Inven tive examp le 8 | 939 | 932 | 554 | 96 | 550 | 5 | 441 | |
| Inven tive examp le 9 | 940 | 953 | 533 | 102 | 525 | 5 | 446 | |
| Compa rativ e examp le 1 | 902 | 949 | 559 | 86 | 553 | 8 | 449 | |
| Compa rativ e examp le 2 | 935 | 935 | 531 | 101 | 526 | 8 | 458 | |
| Compa rativ e examp le 3 | 933 | 914 | 551 | 96 | 545 | 8 | 428 | |
| Compa rativ e examp le 4 | 924 | 953 | 584 | 85 | 576 | 8 | 466 | |
| Compa rativ e examp le 5 | 912 | 941 | 550 | 91 | 541 | 8 | 439 | |
| Compa rativ e examp le 6 | 936 | 924 | 573 | 91 | 567 | 6 | 455 | |
| Compa rativ e examp le 7 | 918 | 938 | 562 | 89 | 555 | 6 | 449 | |
| Compa rativ e examp le 8 | 927 | 939 | 578 | 87 | 571 | 6 | 463 | |
| Compa rativ e examp le 9 | 923 | 947 | 585 | 85 | 570 | 8 | 465 | |
| Compa rativ e examp le 10 | 931 | 945 | 562 | 92 | 565 | 8 | 477 | |
| Compa rativ e examp le 11 | 880 | 892 | 568 | 78 | 563 | 6 | 418 | |
| Compa rativ e examp le 12 | 924 | 949 | 670 | 64 | 635 | 6 | 425 | |
| Compa rativ e examp le 13 | 924 | 949 | 562 | 91 | 556 | 15 | 441 | |
| Compa rativ e examp le 14 | 928 | 953 | 610 | 80 | 558 | 0 | 311 | |
| Compa rativ e examp le 15 | 921 | 946 | 616 | 76 | 599 | 8 | 550 | |

Relational expression 3 is T* - T+225[C]^{0.5}+17[Mn]-34[Si]-20[Mo]-41[V], and the intermediate temperature refers to an intermediate point between the primary cooling termination temperature and the secondary cooling initiation temperature.

**[Table 3]**

| Classif ication | Microstructure | | | | | Rolled sheet properties | | | | |
|---|---|---|---|---|---|---|---|---|---|---|
| | F | B | M+MA | RA | ∑N_{PPT} | TS | El | HER | TS×El | TS×HE R |
| | | | | | | (MPa) | (%) | (%) | (MPa% ) | (MPa% ) |
| Inventi ve example 1 | 5 | 77 | 8 | 10 | 231 | 1240 | 17 | 29 | 21080 | 35960 |
| Inventi ve example 2 | 6 | 76 | 9 | 9 | 192 | 1221 | 17 | 27 | 20757 | 32967 |
| Inventi ve example 3 | 9 | 73 | 7 | 11 | 217 | 1217 | 18 | 29 | 21906 | 35293 |
| Inventi ve example 4 | 6 | 77 | 6 | 11 | 312 | 1249 | 17 | 26 | 21233 | 32474 |
| Inventi ve example 5 | 7 | 76 | 7 | 10 | 292 | 1283 | 16 | 25 | 20528 | 32075 |
| Inventi ve example 6 | 6 | 79 | 6 | 9 | 258 | 1255 | 16 | 24 | 20080 | 30120 |
| Inventi ve example 7 | 9 | 77 | 5 | 9 | 353 | 1211 | 18 | 28 | 21798 | 33908 |
| Inventi ve example 8 | 7 | 77 | 6 | 10 | 501 | 1253 | 17 | 24 | 21301 | 30072 |
| Inventi ve example 9 | 9 | 75 | 7 | 9 | 275 | 1209 | 18 | 26 | 21762 | 31434 |
| Compara tive example 1 | 5 | 63 | 15 | 17 | 184 | 1297 | 16 | 19 | 20752 | 24643 |
| Compara tive example 2 | 25 | 70 | 4 | 1 | 246 | 1098 | 20 | 21 | 21960 | 23058 |
| Compara tive example 3 | 14 | 72 | 5 | 9 | 481 | 1021 | 24 | 18 | 24504 | 18378 |
| Compara tive example 4 | 23 | 68 | 5 | 4 | 295 | 1150 | 19 | 17 | 21850 | 19550 |
| Compara tive example 5 | 5 | 71 | 11 | 13 | 282 | 1310 | 16 | 19 | 20960 | 24890 |
| Compara tive example 6 | 17 | 76 | 4 | 3 | 326 | 1137 | 20 | 20 | 22740 | 22740 |
| Compara tive example 7 | 6 | 78 | 6 | 10 | 264 | 1267 | 17 | 22 | 21539 | 27874 |
| Compara tive example 8 | 14 | 69 | 8 | 9 | 309 | 1176 | 21 | 21 | 24696 | 24696 |
| Compara tive example 9 | 5 | 79 | 6 | 10 | 125 | 1242 | 16 | 23 | 19872 | 28566 |
| Compara tive example 10 | 7 | 85 | 5 | 3 | 6735 | 1375 | 11 | 22 | 15125 | 30250 |
| Compara tive example 11 | 25 | 65 | 5 | 5 | 201 | 1009 | 22 | 24 | 22198 | 24216 |
| Compara tive example 12 | 35 | 56 | 4 | 5 | 5839 | 869 | 19 | 19 | 16511 | 16511 |
| Compara tive example 13 | 43 | 49 | 4 | 4 | 5763 | 821 | 18 | 19 | 14778 | 15599 |
| Compara tive example 14 | 1 | 85 | 12 | 2 | 17 | 1279 | 16 | 21 | 20464 | 26859 |
| Compara tive example 15 | 36 | 60 | 1 | 3 | 5714 | 1085 | 14 | 24 | 15190 | 26040 |

(In Table 3, F: ferrite, B: bainite, M: martensite, MA: Martensite-Austenite constituents, RA: retained austenite. ∑NPPT: the number of precipitates in ferrite present within 100µm from a retained austenite grain boundary per unit area 1 mm²).

As in Table 3, when the composition and manufacturing conditions of the present disclosure were satisfied, high strength of 1180 MPa or more was obtained, TSXEl was 20, 000 MPa% or more, and TSXHER was 30, 000 MPa%, thereby securing excellent formability.

FIG. 1 is a graph illustrating a distribution of TSXEl and TSXHER of inventive examples and comparative examples. Referring to FIG. 1, it has been indicated that excellent physical properties were secured in overall invention examples that satisfied the conditions suggested in the present disclosure.

FIGS. 2 (a) and (b) are images of microstructures of inventive example 7 and comparative example 2, respectively, obtained using an SEM. In inventive example 7, ferrite (F) and retained austenite (RA) were partially included in addition to bainite (B) as a main phase, whereas in comparative example 2, excessive ferrite (F) was formed. Thus, it has been indicated that, in comparative example 2, strength suggested in the present disclosure was not secured.

FIGS. 3(a), (b), and (c) illustrate precipitation formation behavior in a structure adjacent to retained austenite in comparative example 14, inventive example 7 and comparative example 15, respectively. In FIG. 3 (a), it has been indicated that, due to excessive formation of bainite, precipitates in the structure adjacent to retained austenite were rarely formed, whereas, in (c), the secondary cooling was not sufficient, such that excessive precipitates were formed in the structure adjacent to retained austenite, and accordingly, the carbon content for securing stability of retained austenite was insufficient, and elongation was not sufficiently secured.

As shown in Table 3, in comparative examples 1 to 10, the composition of the steel sheet and relational expression 1 or 2 did not satisfy the appropriate range suggested in the present disclosure, and the physical properties suggested in the present disclosure were not secured.

In particular, in comparative examples 9 and 10, the contents of Mo, Ti, Nb, and V were beyond the range suggested in the present disclosure, such that the number of precipitates in a structure adjacent to retained austenite was beyond the effective range suggested in the present disclosure, and accordingly, excellent physical properties was not secured.

In comparative examples 11 to 15, each component satisfied the effective range of the present disclosure, but the finishing temperature after hot rolling and cooling conditions were beyond the effective range suggested in the present disclosure. In these cases, it has been indicated that TSXEl and TSXHER suggested in the present disclosure were not secured.

## Claims

1. A high strength hot-rolled steel sheet having excellent formability, comprising:
by weight%, 0.1-0.15% of C, 2.0-3.0% of Si, 0.8-1.5% of Mn, 0.001-0.05% of P, 0.001-0.01% of S, 0.01-0.1% of AI, 0.7-1.7% of Cr, 0.0001-0.2% of Mo, 0.02-0.1% of Ti, 0.01-0.03% of Nb, 0.001-0.005% of B, 0.1-0.3% of V, 0.001-0.01% of N, and a balance of Fe and inevitable impurities,
wherein [relational expression 1] and [relational expression 2] are satisfied,
wherein tensile strength (TS) is 1180 MPa or more, a product (TS×EI) of tensile strength and elongation is 20,000 MPa% or more, and a product (TS×HER) of tensile strength and hole expandability is 30,000 MPa% or more, and
wherein a microstructure of the hot-rolled steel sheet includes, by an area fraction, 5-15% of ferrite, 5-20% of retained austenite, and 10% or less of inevitable structure, in addition to a bainite matrix structure, $\begin{matrix}20 \leq H γ \leq 50 \\ H γ = 194.5 - \left(428\left[C\right]+11\left[Si\right]+45\left[Mn\right]+35\left[Cr\right]-10\left[Mo\right]-107\left[Ti\right]-56\left[Nb\right]-70\left[V\right]\right)\end{matrix}$
where [elemental symbol] indicates a content in weight% of each element, $\begin{matrix}0.7 \leq {a}_{p} \leq 3.5 \\ {a}_{p} = \left(\left[Mo\right]+\left[Ti\right]+\left[Nb\right]+\left[V\right]\right) \times {\left[C\right]}^{- 1}\end{matrix}$
where [elemental symbol] indicates a content in weight% of each element, wherein the mechanical properties and the microstructure is measured as defined in the description.

2. The high strength hot-rolled steel sheet of claim 1, wherein ferrite has an average hardness value of 200Hv or more.

3. The high strength hot-rolled steel sheet of claim 1, wherein the inevitable structure is one or more of martensite, martensite austenite constituent (MA), and austenite, measured as defined in the description.

4. The high strength hot-rolled steel sheet of claim 1, wherein, in the hot-rolled steel sheet, the number of precipitates having a diameter of 5 nm or more in ferrite present within 100µm from a retained austenite grain boundary in the microstructure is 5×10ⁿ/mm², wherein 1≤n≤3.

5. The high strength hot-rolled steel sheet of claim 4, wherein the precipitate is carbide or nitride including one or more of Mo, Ti, Nb and V.

6. A method for manufacturing the high strength hot-rolled steel sheet having excellent workability of claim 1, the method comprising:
heating a steel slab including, by weight%, 0.1-0.15% of C, 2.0-3.0% of Si, 0.8-1.5% of Mn, 0.001-0.05% of P, 0.001-0.01% of S, 0.01-0.1% of AI, 0.7-1.7% of Cr, 0.0001-0.2% of Mo, 0.02-0.1% of Ti, 0.01-0.03% of Nb, 0.001-0.005% of B, 0.1-0.3% of V, 0.001-0.01% of N, and a balance of Fe and inevitable impurities and satisfying [relational expression 1] and [relational expression 2] as below at 1180-1300°C;
starting hot rolling of the heated slab at Ar3 or higher, and finishing hot rolling the slab under a condition satisfying [Relational expression 3] as below;
performing cooling as primary cooling at a cooling rate of 20-400°C/s to a temperature range of 500-600°C after the hot rolling;
performing cooling as secondary cooling to a temperature range of 350-500°C after the primary cooling; and
performing coiling at a temperature of 350-500°C, $\begin{matrix}20 \leq H γ \leq 50 \\ H γ = 194.5 - \left(428\left[C\right]+11\left[Si\right]+45\left[Mn\right]+35\left[Cr\right]-10\left[Mo\right]-107\left[Ti\right]-56\left[Nb\right]-70\left[V\right]\right)\end{matrix}$
where [elemental symbol] indicates a content in weight% of each element, $\begin{matrix}0.7 \leq {a}_{p} \leq 3.5 \\ {a}_{p} = \left(\left[Mo\right]+\left[Ti\right]+\left[Nb\right]+\left[V\right]\right) \times {\left[C\right]}^{- 1}\end{matrix}$
where [elemental symbol] indicates a content in weight% of each element, $\begin{matrix}900 \leq {T}^{∗} \leq 960 \\ {T}^{∗} = T + 225 {⌈ C ⌉}^{0.5} + 17 ⌈ Mn ⌉ - 34 ⌈ Si ⌉ - 20 ⌈ Mo ⌉ - 41 ⌈ V ⌉\end{matrix}$
where "T" indicates a hot finishing rolling temperature (FDT), and [elemental symbol] indicates a content in weight% of each element.

7. The method of claim 6, wherein a secondary cooling rate is 0.5-70°C/s.

8. The method of claim 6, wherein the method further includes performing extremely slow cooling at a cooling rate of 0.05-4.0°C/s for 12 seconds or less, after the primary cooling.

9. The method of claim 6, wherein the method further includes performing natural cooling to a temperature range of room temperature-200°C and a process of leveling, calibrating, and pickling, after the coiling.

10. The method of claim 6, wherein the method further includes performing heating to a temperature of 600°C or less and plating on the hot-rolled steel sheet.

## Patentansprüche

1. Hochfestes warmgewalztes Stahlblech mit ausgezeichneter Formbarkeit, umfassend:
in Gewichtsprozent 0,1 bis 0,15 % C, 2,0 bis 3,0 % Si, 0,8 bis 1,5 % Mn, 0,001 bis 0,05 % P, 0,001 bis 0,01 % S, 0,01 bis 0,1 % Al, 0,7 bis 1,7 % Cr, 0,0001 bis 0,2 % Mo, 0,02 bis 0,1 % Ti, 0,01 bis 0,03 % Nb, 0,001 bis 0,005 % B, 0,1 bis 0,3 % V, 0,001 bis 0,01 % N und einen Rest aus Fe und unvermeidlichen Verunreinigungen,
wobei [Beziehungsausdruck 1] und [Beziehungsausdruck 2] erfüllt sind,
wobei die Zugfestigkeit (TS) 1180 MPa oder mehr beträgt, ein Produkt (TS × El) aus Zugfestigkeit und Dehnung 20 000 MPa% oder mehr beträgt und ein Produkt (TS × HER) aus Zugfestigkeit und Lochdehnbarkeit 30 000 MPa% oder mehr beträgt und
wobei eine Mikrostruktur des warmgewalzten Stahlblechs zusätzlich zu einer Bainit-Matrixstruktur einen Flächenanteil von 5 bis 15 % Ferrit, 5 bis 20 % Restaustenit und 10 % oder weniger an unvermeidlicher Struktur beinhaltet, $\begin{matrix}20 \leq H γ \leq 50 \\ H γ = 194,5 - \left(\begin{matrix}428 \left[C\right] + 11 \left[Si\right] + 45 \left[Mn\right] + 35 \left[Cr\right] - 10 \left[Mo\right] - 107 \left[Ti\right] - \\ 56 \left[Nb\right] - 70 \left[V\right]\end{matrix}\right)\end{matrix}$
wobei [Elementsymbol] einen Gehalt jedes Elements in Gewichtsprozent angibt, $\begin{matrix}0,7 \leq {a}_{p} \leq 3,5 \\ {a}_{p} = \left(\left[Mo\right]+\left[Ti\right]+\left[Nb\right]+\left[V\right]\right) \times {\left[C\right]}^{- 1}\end{matrix}$
wobei [Elementsymbol] einen Gehalt jedes Elements in Gewichtsprozent angibt,
wobei die mechanischen Eigenschaften und die Mikrostruktur wie in der Beschreibung definiert gemessen werden.

2. Hochfestes warmgewalztes Stahlblech nach Anspruch 1, wobei Ferrit einen durchschnittlichen Härtewert von 200 Hv oder mehr aufweist.

3. Hochfestes warmgewalztes Stahlblech nach Anspruch 1, wobei es sich bei der unvermeidlichen Struktur um eines oder mehreres aus Martensit, Martensit-Austenit-Komponenten (MA) und Austenit handelt, die wie in der Beschreibung definiert gemessen werden.

4. Hochfestes warmgewalztes Stahlblech nach Anspruch 1, wobei in dem warmgewalzten Stahlblech die Anzahl an Ausfällungen mit einem Durchmesser von 5 nm oder mehr in Ferrit, die innerhalb von 100 µm von einer Restaustenit-Korngrenze in der Mikrostruktur vorhanden sind, 5×10ⁿ/mm² beträgt, wobei 1 ≤ n ≤ 3.

5. Hochfestes warmgewalztes Stahlblech nach Anspruch 4, wobei die Ausfällung Carbid oder Nitrid ist, das eines oder mehreres aus Mo, Ti, Nb und V beinhaltet.

6. Verfahren zur Herstellung des warmgewalzten Stahlblechs mit ausgezeichneter Bearbeitbarkeit nach Anspruch 1, wobei das Verfahren Folgendes umfasst:
Erwärmen einer Stahlbramme, die in Gewichtsprozent 0,1 bis 0,15 % C, 2,0 bis 3,0 % Si, 0,8 bis 1,5 % Mn, 0,001 bis 0,05 % P, 0,001 bis 0,01 % S, 0,01 bis 0,1 % Al, 0,7 bis 1,7 % Cr, 0,0001 bis 0,2 % Mo, 0,02 bis 0,1 % Ti, 0,01 bis 0,03 % Nb, 0,001 bis 0,005 % B, 0,1 bis 0,3 % V, 0,001 bis 0,01 % N und einen Rest aus Fe und unvermeidlichen Verunreinigungen beinhaltet und [Beziehungsausdruck 1] und [Beziehungsausdruck 2], wie nachstehend angegeben, erfüllt, auf 1180 bis 1300 °C;
Beginnen des Warmwalzens der erwärmten Bramme bei Ar3 oder höher und Beenden des Warmwalzens der Bramme unter einer Bedingung, die den nachstehenden [Beziehungsausdruck 3] erfüllt;
Durchführen eines Abkühlens als primäres Abkühlen mit einer Abkühlungsgeschwindigkeit von 20 bis 400 °C/s auf einen Temperaturbereich von 500 bis 600 °C nach dem Warmwalzen;
Durchführen eines Abkühlens als sekundäres Abkühlen auf einen Temperaturbereich von 350 bis 500 °C nach dem primären Abkühlen; und
Durchführen eines Wickelns bei einer Temperatur von 350 bis 500 °C, $\begin{matrix}20 \leq H γ \leq 50 \\ H γ = 194,5 - \left(\begin{matrix}428 \left[C\right] + 11 \left[Si\right] + 45 \left[Mn\right] + 35 \left[Cr\right] - 10 \left[Mo\right] - 107 \left[Ti\right] - \\ 56 \left[Nb\right] - 70 \left[V\right]\end{matrix}\right)\end{matrix}$
wobei [Elementsymbol] einen Gehalt jedes Elements in Gewichtsprozent angibt, $\begin{matrix}0,7 \leq {a}_{p} \leq 3,5 \\ ap = \left(\left[Mo\right]+\left[Ti\right]+\left[Nb\right]+\left[V\right]\right) \times {\left[C\right]}^{- 1}\end{matrix}$
wobei [Elementsymbol] einen Gehalt jedes Elements in Gewichtsprozent angibt, $\begin{matrix}900 \leq T * \leq 960 \\ T * = T + 225 {\left[C\right]}^{0,5} + 17 \left[Mn\right] - 34 \left[Si\right] - 20 \left[Mo\right] - 41 \left[V\right]\end{matrix}$
wobei "T" eine Warmfertigwalztemperatur (FDT) angibt und [Elementsymbol] einen Gehalt jedes Elements in Gewichtsprozent angibt.

7. Verfahren nach Anspruch 6, wobei eine sekundäre Abkühlungsgeschwindigkeit 0,5 bis 70 °C/s beträgt.

8. Verfahren nach Anspruch 6, wobei das Verfahren ferner das Durchführen eines extrem langsamen Abkühlens mit einer Abkühlungsgeschwindigkeit von 0,05 bis 4,0 °C/s während 12 Sekunden oder weniger nach dem primären Abkühlen beinhaltet.

9. Verfahren nach Anspruch 6, wobei das Verfahren ferner das Durchführen eines natürlichen Abkühlens auf einen Temperaturbereich von Raumtemperatur bis 200 °C und einen Vorgang des Nivellierens, Kalibrierens und Beizens nach dem Wickeln beinhaltet.

10. Verfahren nach Anspruch 6, wobei das Verfahren ferner das Durchführen eines Erwärmens auf eine Temperatur von 600 °C oder weniger und das Plattieren des warmgewalzten Stahlblechs beinhaltet.

## Revendications

1. Tôle d'acier laminée à chaud à haute résistance, présentant une excellente aptitude au formage, comprenant :
en % en poids, 0,1 à 0,15 % de C, 2,0 à 3,0 % de Si, 0,8 à 1,5 % de Mn, 0,001 à 0,05 % de P, 0,001 à 0,01 % de S, 0,01 à 0,1 % d'Al, 0,7 à 1,7 % de Cr, 0,0001 à 0,2 % de Mo, 0,02 à 0,1 % de Ti, 0,01 à 0,03 % de Nb, 0,001 à 0,005 % de B, 0,1 à 0,3 % de V, 0,001 à 0,01 % de N, et un reste de Fe et d'impuretés inévitables,
dans laquelle l' [expression relationnelle 1] et l' [expression relationnelle 2] sont satisfaites,
dans laquelle la résistance à la traction (TS) est de 1180 MPa ou plus, un produit (TS × El) de la résistance à la traction et de l'allongement est de 20 000 MPa % ou plus, et un produit (TS × HER) de la résistance à la traction et de l'expansion du trou est de 30 000 MPa % ou plus, et
dans laquelle une microstructure de la tôle d'acier laminée à chaud inclut, par fraction d'aire, 5 à 15 % de ferrite, 5 à 20 % d'austénite retenue, et 10 % ou moins de structure inévitable, en plus d'une structure matricielle de bainite, $\begin{matrix}20 \leq Hy \leq 50 \\ Hy = 194,5 - \left(\begin{matrix}428 \left[C\right] + 11 \left[Si\right] + 45 \left[Mn\right] + 35 \left[Cr\right] - \\ 10 \left[Mo\right] - 107 \left[Ti\right] - 56 \left[Nb\right] - 70 \left[V\right]\end{matrix}\right)\end{matrix}$
où [symbole élémentaire] indique une teneur en % en poids de chaque élément, $\begin{matrix}0.7 \leq {a}_{p} \leq 3,5 \\ {a}_{p} = \left(\left[Mo\right]+\left[Ti\right]+\left[Nb\right]+\left[V\right]\right) \times {\left[C\right]}^{- 1}\end{matrix}$
où [symbole élémentaire] indique une teneur en % en poids de chaque élément, dans laquelle les propriétés mécaniques et la microstructure sont mesurées comme défini dans la description.

2. Tôle d'acier laminée à chaud à haute résistance selon la revendication 1, dans laquelle la ferrite a une valeur de dureté moyenne de 200 Hv ou plus.

3. Tôle d'acier laminée à chaud à haute résistance selon la revendication 1, dans laquelle la structure inévitable est un ou plusieurs parmi de la martensite, un constituant martensite-austénite (MA), et de l'austénite, mesurée comme défini dans la description.

4. Tôle d'acier laminée à chaud à haute résistance selon la revendication 1, dans laquelle, dans la tôle d'acier laminée à chaud, le nombre de précipités ayant un diamètre de 5 nm ou plus dans la ferrite présente au sein de 100 µm d'un joint de grains d'austénite retenue dans la microstructure est de 5 × 10ⁿ/mm², dans laquelle 1 ≤ n ≤ 3.

5. Tôle d'acier laminée à chaud à haute résistance selon la revendication 4, dans laquelle le précipité est un carbure ou un nitrure incluant un ou plusieurs parmi Mo, Ti, Nb et V.

6. Procédé de fabrication de la tôle d'acier laminée à chaud à haute résistance présentant une excellente aptitude au façonnage de la revendication 1, le procédé comprenant :
le chauffage d'une brame d'acier incluant, en % en poids, 0,1 à 0,15 % de C, 2,0 à 3,0 % de Si, 0,8 à 1,5 % de Mn, 0, 001 à 0,05 % de P, 0, 001 à 0, 01 % de S, 0, 01 à 0, 1 % d'Al, 0,7 à 1,7 % de Cr, 0, 0001 à 0,2 % de Mo, 0,02 à 0,1 % de Ti, 0,01 à 0,03 % de Nb, 0,001 à 0,005 % de B, 0,1 à 0,3 % de V, 0,001 à 0,01 % de N, et un reste de Fe et d'impuretés inévitables et satisfaisant l'[expression relationnelle 1] et l' [expression relationnelle 2] comme ci-dessous à 1180 à 1300 °C ;
le démarrage du laminage à chaud de la brame chauffée à Ar3 ou plus, et le laminage à chaud de finition de la brame dans des conditions satisfaisant l' [expression relationnelle 3] comme ci-dessous ;
la réalisation d'un refroidissement en tant que refroidissement primaire à une vitesse de refroidissement de 20 à 400 °C/s jusqu'à une plage de températures de 500 à 600 °C après le laminage à chaud ;
la réalisation d'un refroidissement en tant que refroidissement secondaire jusqu'à une plage de températures de 350 à 500 °C après le refroidissement primaire ; et
la réalisation d'un bobinage à une température de 350 à 500 °C, $\begin{matrix}20 \leq Hy \leq 50 \\ Hy = 194,5 - \left(\begin{matrix}428 \left[C\right] + 11 \left[Si\right] + 45 \left[Mn\right] + 35 \left[Cr\right] - \\ 10 \left[Mo\right] - 107 \left[Ti\right] - 56 \left[Nb\right] - 70 \left[V\right]\end{matrix}\right)\end{matrix}$
où [symbole élémentaire] indique une teneur en % en poids de chaque élément, $\begin{matrix}0,7 \leq {a}_{p} \leq 3,5 \\ {a}_{p} = \left(\left[Mo\right]+\left[Ti\right]+\left[Nb\right]+\left[V\right]\right) \times {\left[C\right]}^{- 1}\end{matrix}$
où [symbole élémentaire] indique une teneur en % en poids de chaque élément, $\begin{matrix}900 \leq {T}^{∗} \leq 960 \\ {T}^{∗} = T + 225 {\left[C\right]}^{0,5} + 17 \left[Mn\right] - 34 \left[Si\right] - 20 \left[Mo\right] - 41 \left[V\right]\end{matrix}$
où « T » indique une température de laminage à chaud de finition (FDT), et [symbole élémentaire] indique une teneur en % en poids de chaque élément.

7. Procédé selon la revendication 6, dans lequel une vitesse de refroidissement secondaire est de 0,5 à 70 °C/s.

8. Procédé selon la revendication 6, le procédé incluant en outre la réalisation d'un refroidissement extrêmement lent à une vitesse de refroidissement de 0,05 à 4,0 °C/s pendant 12 secondes ou moins, après le refroidissement primaire.

9. Procédé selon la revendication 6, le procédé incluant en outre la réalisation d'un refroidissement naturel jusqu'à une plage de températures de la température ambiante à 200 °C, et d'un processus de nivelage, d'étalonnage et de décapage, après le bobinage.

10. Procédé selon la revendication 6, le procédé incluant en outre la réalisation d'un chauffage jusqu'à une température de 600 °C ou moins et d'un placage sur la tôle d'acier laminée à chaud.
